

Nov. 18, 1947.

V. N. BORSOFF ET AL

2,430,857

FOAM INHIBITED OIL

Filed July 14, 1942

2 Sheets—Sheet 1



Fig. 1

INVENTORS

Victor N. Borsoff

James O. Clayton

By

*J. Adams*

Attorney

Nov. 18, 1947.

V. N. BORSOFF ET AL

2,430,857

FOAM INHIBITED OIL

Filed July 14, 1942

2 Sheets-Sheet 2



Fig. 2



Fig. 3

INVENTORS

Victor N. Borsoff

James O. Clayton

By Adams  
Attorney

## UNITED STATES PATENT OFFICE

2,430,857

## FOAM INHIBITED OIL

Victor N. Borsoff and James O. Clayton, Berkeley, Calif., assignors, by mesne assignments, to California Research Corporation, San Francisco, Calif., a corporation of Delaware

Application July 14, 1942, Serial No. 450,886

20 Claims. (Cl. 252—52)

1

This invention relates to oils inhibited against the formation of a stable bubble foam and to a method of inhibiting the foam formation tendency of oils.

On mixing oil with air, a certain amount of foam may be created. The amount of foam will depend, among other things, upon the character of the oil and the type of service in which it is employed. Thus most base mineral oils, that is mineral oils uncompounded with a chemical additive, do not readily form foam, at least under ordinary service conditions. Many compounded oils tend to produce a more stable foam than the base oils from which they are compounded. Thus petroleum lubricating oils compounded with metal naphthenates, higher metal alcoholates, higher metal alkyl phenates and metal salts of higher fatty acids foam more than the corresponding base oils. Many other additives cause more foam to be produced by oils to which they are added than is formed by the base oils.

Oil foaming, even with compounded oils which display the greatest tendency to foam, is not always troublesome. Under conditions of little or no agitation, for example, trouble due to foaming is encountered, if at all, only in very exceptional cases. On the other hand, certain drastic types of service, involving extremely violent intermixture of oil and air or combustion gases, may produce an objectionable amount of foam with many oils. Between the extremes, however, of service causing little foaming of any oil and service causing much foaming of many oils, there are types of service and certain oils which, when used in combination, cause considerable difficulty. As stated, certain compounded oils exhibit a greater tendency to foam than the base oils, and when these compounded oils are used in certain types of lubrication systems, involving greater agitation of the oil and greater intermixture with gases than the ordinary crankcase lubrication of automobiles, the greatest practical difficulty is encountered.

Illustrative of the type of lubrication system which, when used with compounded lubricating oils having a strong tendency to foam, causes practical difficulty, is the dry sump lubrication system employed in many aircraft engines. In this system, oil from the moving parts of the motor is collected in the crankcase and pumped from there to an external tank or sump by a scavenging pump. Oil from this sump is pumped back to the motor in the usual manner by an oil pump. The foaming difficulty arises from the fact that the scavenging pump operates at excess capacity; it pumps faster than required to pump all of the available oil in the crankcase. It therefore pumps a great deal of air along with the oil, and this at a rapid rate, and the result is entrainment of air in the oil and the formation of foam. As a consequence, excessive foaming oc-

2

curs when oils such as the aforementioned compounded oils are used and oil is lost through the breather pipes, insufficient lubrication results because of the presence of air in the oil supplied to the motor, and other disadvantages result.

Oil also forms a more persistent foam if it contains water (as in solution) and is then heated and suddenly subjected to a very low pressure, as, for instance, in an airplane engine climbing from a low altitude to 40,000 feet at a high speed.

In other instances, as in the lubrication of gears with heavy oils, foaming difficulties may also be encountered.

It is an object achieved by the present invention to inhibit the foaming of oils.

It is a further object achieved by the present invention to inhibit the foaming of compounded mineral lubricating oils.

It is a still further and a particular object achieved by the present invention to obviate the problem of excessive foaming of compounded mineral lubricating oils when used in types of lubrication service involving severe conditions of intermixture of oil and gases.

Other objects achieved by the invention will be apparent from the following description and from the claims.

We have discovered that foaming of oils can be inhibited by incorporating therein a small amount of a compound containing not less than about 15% by weight of oxygen and represented by the formula—



wherein A is an aromatic nucleus, X is an oxygen-containing substituent, R is a substituent selected from the group consisting of hydrogen, alkyl, aryl, aralkyl and cyclo-alkyl radicals, a is a whole number at least equal to 1 and b is zero or a whole number. The aromatic nucleus A may contain other substituents in addition to X and OR.

We have found that such oxygen-containing substituted aromatic compounds are effective in reducing foaming even when used in very small amounts, and that they are highly effective in inhibiting the foaming of compounded lubricating oils when subjected to extreme agitation and intermixture with gases. They are, however, not limited in their effectiveness to compounded oils but may be used to advantage wherever troublesome foaming of oils is encountered. Certain of the foam inhibitors of the invention are more effective than others for a given set of conditions,

whereas for another set of conditions a different group of inhibitors will be found to be superior. Simple experiment will enable one to select the best inhibitor for the purpose at hand.

The class of inhibitors falling within the scope of the present invention will first be illustrated with reference to the component parts A, X and

(OR) and then with reference to specific examples of such inhibitors.

The component A, which is an aromatic nucleus, may be, for example, the benzene nucleus or a polycyclic aromatic nucleus such as the naphthalene nucleus, and the aromatic nucleus may be substituted, in addition to the substituents X and OR, by any one or more of numerous groups, such as alkyl, halogen, amino, nitro, etc.

The component X, which must contain at least one oxygen atom, may be, for example, an hydroxyl group; an ether group; any one of the groups —COOR, RCOO—, and —R'—COOR, wherein R and R' may be hydrocarbon or substituted hydrocarbon residues; a ketone or an aldehyde group; a carbinol group, etc.

The component OR may be lacking entirely (b=zero) but preferably it is present (b=1 or greater); that is, our foam inhibitors preferably contain a plurality of oxygen-containing substituents attached to the aromatic nucleus A. Typical examples of the component OR are hydroxyl, alkoxy, aryloxy, and cyclo-alkoxy groups. Where R is a hydrocarbon radical it may contain substituent groups including oxygen-containing substituent groups such as hydroxyl, aldehyde, ketone, carbinol and carboxy groups.

Specific examples typifying the class of inhibitors which we have found to be effective are the following:

Still further examples of foam inhibitors are as follows:

#### Carboxy acids

Amylbenzoic acid  
Octylsalicylic acid

#### Esters

Methyl benzoate  
Ethyl benzoate  
Propyl benzoate  
Butyl benzoate  
Amyl benzoate  
Ethyl salicylate  
Propyl salicylate  
Butyl salicylate  
Octyl salicylate  
Amyl p-hydroxybenzoate  
Methyl m-hydroxybenzoate  
Octyl gallate  
Amyl o-acetylbenzoate  
Ethyl p-benzoylbenzoate  
Diamyl salicylate  
Amyl-o-pyrocatechinate  
Hexyl beta-resorcylate  
Propyl gentisate  
Ethyl veratrate  
Ethyl hemillitate  
Ethyl 2,4-xylate  
Ethyl mesitylenate  
Amyl o-ethoxybenzoate

#### Phenols

Phenol  
Cresol  
25 Hydroquinone  
Resorcinol  
Pyrocatechol  
Methylpyrocatechol  
Cresocinol  
Toluhydroquinone  
Methyresorcinol  
Orcinol  
Dimethylresorcinol  
Dimethylhydroquinone

Ethylresorcinol  
Propylresorcinol  
Butylresorcinol  
Amylresorcinol  
Hexylresorcinol  
Ethylhydroquinone  
Ethylpyrocatechol  
Hexylpyrogallol  
Hexylphloroglucinol  
Hexylhydroxyhydroquinone  
Dihydroxynaphthalenes  
Anthracenediol

| Inhibitor                 | Molecular Structure | Molecular Weight | Per Cent by Weight of Oxygen |
|---------------------------|---------------------|------------------|------------------------------|
| Benzaldehyde.....         |                     | 106              | 15.1                         |
| Saligenin.....            |                     | 124              | 25.8                         |
| Methyl salicylate.....    |                     | 152              | 31.6                         |
| Resorcinol monoacetate... |                     | 152              | 31.6                         |
| Benzoyl acetone.....      |                     | 162              | 19.8                         |
| Amyl salicylate.....      |                     | 208              | 23.1                         |
| Phenyl salicylate.....    |                     | 214              | 22.5                         |
| Naphthyl salicylate.....  |                     | 264              | 18.4                         |

*Ethers*

|                               |                               |
|-------------------------------|-------------------------------|
| Methyl phenyl ether           | Pyrocatechol monopropyl ether |
| Guaiacol                      | Resorcinol monopropyl ether   |
| Resorcinol monomethyl ether   | Hydroquinone monopropyl ether |
| Hydroquinone monomethyl ether | Pyrocatechol monoamyl ether   |
| ether                         | Resorcinol monoamyl ether     |
| Veratrol                      | Hydroquinone monoamyl ether   |
| Resorcinol dimethyl ether     | Pyrocatechol dibutyl ether    |
| Hydroquinone dimethyl ether   | Phloroglucinol triethyl ether |
| Guaethol                      | Pyrogallol tributyl ether     |
| Resorcinol monoethyl ether    | Dimethoxynaphthalene          |
| Hydroquinone monoethyl ether  |                               |

*Aldehydes and ketones*

|                            |                                    |
|----------------------------|------------------------------------|
| Amylquinone                | 1-hydroxy-2-naphthyl methyl ketone |
| Salicylaldehyde            | Octylanthragallol                  |
| Amyl-p-hydroxybenzaldehyde |                                    |
| Furyl phenyl ketone        |                                    |

Preferably we use as foam inhibitors oxygen-containing aromatic compounds containing not less than about 15 per cent by weight of oxygen, and having a molecular weight not higher than about 270. We also prefer to use as inhibitors those compounds which are soluble in mineral oil to the extent used. Less soluble inhibitors are more likely to be removed by filtration or to settle out on standing. However, oil solubility is not essential to effectiveness in reducing foam and a solubility of the order of 0.001 per cent by weight based on the oil is adequate.

The inhibitors of our invention may be advantageously used in a wide variety of oils, including naphthenic base, paraffin base and mixed base mineral oils, in synthetic oils, and in oils of viscosity ranging from 40 SSU or lower at 210° F. to 150 SSU or higher at 210° F.

Preferably the foam inhibitors of the present invention are used in the finished oil in an amount equal to about 0.001% to 1 per cent by weight based on the oil. If the oil is a compounded oil containing 0.1 to 5.0 per cent by weight of an additive which promotes foaming, the foam inhibitor is preferably used in an amount equal to about 10 to 200 per cent by weight based on the additive.

Concentrated solutions of foam inhibitor in oil may be prepared. Such concentrates may also contain other compounding agents. By diluting the concentrate with more oil, a finished oil can be produced containing foam inhibitor, or foam inhibitor and other compounding agent or agents in the desired amount. Conveniently, concentrates containing from about 1.0 to 20 per cent by weight of foam inhibitor based on the total concentrate are thus prepared, in cases where the foam inhibitor is sufficiently oil soluble.

The following specific examples will serve to illustrate the advantages and effectiveness of the inhibitors of the invention in reducing foam formation:

**EXAMPLE I**

The foaming qualities of various oils were observed. The base stock was a solvent treated, paraffinic base oil having a viscosity of 120 SSU at 210° F., and a viscosity index of 86. The first oil tested consisted of this base stock alone and the second oil consisted of the base stock compounded with 0.25 per cent by weight of a 2:1 mixture of a calcium alkyl phenate and a calcium cetyl phosphate. The calcium alkyl phenate so used was the salt of an alkyl substituted phenol prepared by condensing butene polymers, having an average molecular weight of about 196, with phenol. The calcium cetyl phosphate so used was the salt prepared from a mixture of monooctyl- and dicetyl-phosphoric acids. The remaining oils each consisted of base stock, 0.25 per cent by weight of the same phenate-phosphate

6 mixture, and 0.1 per cent by weight of a foam inhibitor. The test conditions were as follows:

500 cc. of the oil were placed in a cylindrical metal container 6 inches in diameter by 5 inches high and a "Mix-Master" stirrer of the type used in household kitchens was lowered into the oil. The oil was slowly heated by means of an electric hot plate and the amount of foam produced was measured at various temperatures up to 300° F. The speed of the stirrer was 1100 revolutions per minute. The test results at 275° F., under identical operating conditions except for variation of the oil composition, are set forth in Table I below:

Table I

|                                              | Per cent increase in volume at 275° F. |
|----------------------------------------------|----------------------------------------|
| Uncompounded oil                             | 11                                     |
| Compounded oil                               | 57                                     |
| Compounded oil + 0.1% benzaldehyde           | 29                                     |
| Compounded oil + 0.1% saligenin              | 17                                     |
| Compounded oil + 0.1% methyl salicylate      | 23                                     |
| Compounded oil + 0.1% resorcinol monoacetate | 29                                     |
| Compounded oil + 0.1% benzoyl acetone        | 11                                     |
| Compounded oil + 0.1% amyl salicylate        | 47                                     |
| Compounded oil + 0.1% phenyl salicylate      | 29                                     |
| Compounded oil + 0.1% naphthyl salicylate    | 29                                     |

20 The per cent increase in volume referred to in the above table, and again in Table II below, is arrived at by observing the increase in volume of the mixture of foam and oil over the original volume of oil, dividing the increase by the original volume of oil, and multiplying by 100. It is, therefore, the volume of foam produced reckoned as per cent of the original volume of oil.

**EXAMPLE II**

40 Oils were tested in an apparatus comprising a reservoir adapted to be heated by a hot plate, a sump situated below the reservoir, a drain provided with a regulating valve and leading from the bottom of the reservoir to the sump, and a return conduit connected with the bottom of the sump, provided with a pump, and extending into the reservoir under the surface of the oil therein. Oil, maintained at 200° F. in the reservoir, dropped from the reservoir through the drain to the sump at a rate controlled by the regulating valve. The pump in the return conduit was operated at a capacity three times the rate of flow of oil into the sump; therefore, both oil and air were pumped from the sump to the reservoir and foaming was caused in the reservoir. At the end of each 30 minutes of operation, the volume of foam and oil in the reservoir was observed. The amount of foam was calculated as the per cent increase in volume over the original volume of oil. Under identical operating conditions, various oils produced increases in volume as given in Table II below:

Table II

|                                              | Per cent increase in volume |
|----------------------------------------------|-----------------------------|
| Uncompounded oil                             | 30                          |
| Compounded oil                               | 200+                        |
| Compounded oil + 0.1% benzaldehyde           | 75                          |
| Compounded oil + 0.1% saligenin              | 65                          |
| Compounded oil + 0.1% methyl salicylate      | 65                          |
| Compounded oil + 0.1% resorcinol monoacetate | 85                          |
| Compounded oil + 0.1% benzoyl acetone        | 10                          |
| Compounded oil + 0.1% amyl salicylate        | 85                          |
| Compounded oil + 0.1% phenyl salicylate      | 65                          |

## EXAMPLE III

A 1939 Ford V-8, 85 horsepower engine was thus modified: The bottom of the crankcase was connected to a large glass container and the suction line of the oil pump was connected to the glass container. Oil dropping from the moving parts drained from the crankcase through the pipe to the glass container and was pumped back to the engine from the glass container through the suction line. The air pressure in the crankcase was maintained at 1½ inches of mercury. In this manner air became mixed with the oil draining from the crankcase and produced foam in the glass container, where it could be observed.

Under identical operating conditions a compounded oil, and the same compounded oil plus 0.05 per cent of saligenin, produced the following depths of foam in the glass container:

|                                  | Depth of foam<br>in inches |
|----------------------------------|----------------------------|
| Compounded oil                   | 2.5                        |
| Compounded oil + 0.05% saligenin | 0.5                        |

As stated above, the inhibitors of the invention are not all equally effective in inhibiting foam formation. Some of the inhibitors are less effective than others under all or most conditions. Some inhibitors are the most effective under certain conditions whereas others are the most effective under other conditions. Thus, as shown by the above specific examples, amyl salicylate is among the least effective of the inhibitors both in the open vessel-mechanical stirrer test (Example I) and in the sump test (Example II). However, in both tests it effects a substantial reduction in foaming. Benzoyl acetone is among the most effective foam inhibitors judged by either of these tests.

In addition to effectiveness in reducing foam formation, it is desirable that a foam inhibitor possess certain other desirable properties. Among such additional properties are lack of objectionable odor, at least a slight solubility in lubricating oil, stability at high and at low temperatures, noncorrosiveness to bearings, such as alloy bearings, and good engine performance (that is, the inhibitor should not increase ring sticking, should not increase gum or resin formation on pistons or other hot parts of the engine, and should not increase wear). Also, it is desirable that the inhibitor be not subject to removal on filtering. The best inhibitor is, therefore, one which is highly effective in reducing foaming and which also possesses, in high degree, the desirable properties listed above. Saligenin, or ortho hydroxy benzyl alcohol, is, from this standpoint, the best inhibitor. It is highly effective in reducing foam, it lacks odor when present in mineral lubricating oil in small amount, it is sufficiently soluble in mineral lubricating oil, it is stable at low and at high temperatures, it is not removed by filtration of oil containing it, it is noncorrosive to alloy bearings, and it does not cause deterioration of engine performance.

We have observed that our inhibitors are more effective at elevated temperatures than at lower temperatures. At about the ordinary temperature, the reduction in foaming produced by the inhibitors of the invention is small, although substantial. At about 120° to 150° F. the reduction of foaming begins to be large, and above about 150° F. the reduction in foaming is very large.

The effect of temperature upon foaming of un-

hibited and inhibited oils is shown by Fig. 1 of the accompanying drawings.

In Fig. 1, abscissae represent temperature in degrees Fahrenheit and ordinates represent the volume of foam calculated as percentage on the original volume of oil. Curve A represents the uncompounded oil of Example I, curve B represents the same oil compounded with 0.25 per cent by weight of a 2:1 mixture of calcium alkyl phenate and calcium cetyl phosphate (the same as used in Example I), and curve C represents the same compounded oil containing, in addition to the phenate and phosphate, 0.1 per cent of saligenin. The test conditions were the same as in Example I, except that observations were made at a number of different temperatures.

It will be noted that foaming was great in the case of all three oils at 80° F., though substantially less with oil A (uncompounded oil) and oil C (compounded oil containing saligenin) than with oil B (compounded oil containing no saligenin). As the temperature increased, the foaming of all three oils decreased, but the foaming of oils A and C decreased more rapidly than that of oil B. At about 170° F., however, oil B began to foam more with increase in temperature whereas oils A and C continued to decrease in amount of foaming.

It will be noted that the inhibitor exerted greater effectiveness in reducing foam formation at higher temperatures than at lower temperatures. From the standpoint of foam formation in internal combustion engines this is important. Crankcase temperatures are generally above about 200° F., although the crankcases of some engines operate at temperatures as low as about 150° F. It is at temperatures above about 150° F., especially above about 200° F., that excessive foaming is likely to occur. At these temperatures the inhibitors of our invention are highly effective in reducing foam formation.

The phenate-phosphate mixture referred to above is effective in inhibiting oxidation of lubricating oils and in reducing ring sticking. It is given by way of example of the oil-soluble metal organic salts which are widely used in lubricating oils for such purposes. The tendency of such compounding agents to promote foaming detracts somewhat from their utility, and the obviation of this defect, by the use of our foam inhibitors, is one of the principal objects accomplished by the invention.

It has been found that certain compounded oils which foam excessively also develop surfaces having the characteristics of plastic solids; that is, the surface is highly viscous, yields to and is deformed by a pressure in excess of a minimum yield value, but does not flow freely like a liquid under the force of gravity. This fact has been brought to light through the use of the torsion pendulum. This apparatus and its use to determine surface plasticity and viscosity of aqueous solutions is described by R. E. Wilson and E. D. Ries in "Surface films as plastic solids," Colloid Symposium Monograph, volume I, pages 145-173, published by the Department of Chemistry, University of Wisconsin 1923. The same apparatus and method were used to determine surface plasticity and viscosity of mineral oils.

Thus an SAE 30 blend of 70% Western acid treated naphthenic base oil and 30% Western paraffinic base oil compounded with 0.25% by weight of a 2:1 mixture of a calcium alkyl phenate and a calcium-cetyl phosphate (the same as Example I) was investigated by means of the tor-

sion pendulum. The base oil is a non-foaming oil and the compounded oil exhibits a marked tendency to foam under the conditions of Example I. It was found that at room temperature the surface of the compounded oil, on ageing, became very viscous and similar to a plastic solid. However, when 0.1% of saligenin was dissolved in the compounded oil, a sharp initial rise in the viscosity of a freshly formed surface occurred and the surface became plastic, but after about 40 minutes the viscosity dropped off sharply and then more slowly. The surface became liquid again. The use of 0.2% of saligenin produced a similar result in less time.

A similar experiment at 200° F. revealed that the same compounded oil (lacking foam inhibitor) increased in surface viscosity during the first 2.5 minutes, remained constant for 1 minute and increased sharply between 3.5 and 4.0 minutes, and that after 4 minutes the surface was a plastic solid. On dissolving 0.1% of saligenin in the compounded oil, the surface viscosity-time curve was found to be anomalous for the first 7 minutes, exhibiting sharp drops and subsequent rises in viscosity. After about 9 minutes the surface began to set like a gel and become like a plastic solid, but a plastic solid having a very low yield point.

At both room temperature and 200° F., therefore, a correlation was found between surface viscosity and foaming tendency; the excessively foaming oil formed a surface, on ageing, similar to a plastic solid, but the foam inhibited oil formed a liquid surface on ageing at room temperature or a plastic solid surface of very low yield point on ageing at 200° F.

Therefore, those oils whose surfaces on ageing (a matter of minutes) exhibit the properties of plastic solids with high yield points are excessively foaming oils, while oils whose surfaces on ageing remain liquid or exhibit the properties of plastic solids with very low yield points are not excessively foaming oils. The most probable explanation of these observed phenomena seems to be as follows: All oils, when agitated with air produce foam, which consists of small portions of air each surrounded by a film of oil. In many cases this foam is unstable, probably due to the instability of the film of oil. This film is so fluid that continued agitation and collisions of the foam bubbles with each other and the sides of the vessel and draining of the liquid from the film cause rupture of the film and destruction of the bubbles. In those cases, however, where the oil surface (hence the film of oil enclosing the air in the foam) is a plastic solid, the film is not as easily ruptured because the liquid cannot drain from the film due to capillary forces set up by the plastic solid surfaces, and the foam is stable. The plasticity and stability of the oil film clearly depend, in part at least, upon the nature and amount of solutes in the oil. Thus metal salts such as metal naphthenates, metal soaps of higher fatty acids, higher metal alkyl phenates, metal salts of phosphoric acid partly esterified by long chain alcohols, and higher metal alcoholates are apparently adsorbed by the film of oil and render it more viscous, plastic and tough. We do not wish to infer that this is the only factor influencing foaming or that all foaming is due to the formation of a plastic solid film, but this is one of the principal contributing factors. The inhibitors of this invention, such as saligenin, apparently function by reducing the amount of adsorption of the foam-producing salts in the film, or are themselves adsorbed and counteract the adsorbed foam-producing salts.

Our invention, however, is not limited in its application to those oils which, because of certain salt-like compounding agents, form viscous, plastic surfaces. Our invention is applicable broadly to the inhibition of oil foaming wherever it occurs and comprises the addition of our foam inhibiting agents to any oil which foams excessively.

For the purpose of clarity, the terms "excessive foaming," "excessively foaming," and the like, as applied to oils herein and in the claims, refer to performance under the conditions of the following reproducible test, described with reference to Figs. 2 and 3 of the accompanying drawings. An oil which, when agitated under the conditions of this test at 275° F., increases in volume due to foaming by more than 20 per cent of its original volume, is an "excessively foaming" oil, and oils which foam less than this amount are not "excessively foaming" oils.

500 cc. of oil are placed in a cylindrical flat bottomed container 6" in diameter and 5" high (internal dimensions), the oil in the container is brought to and maintained at 275° F. by any suitable means such as a hot plate or a jacket, and the stirring elements of a "Mix Master" stirrer of the type used in household kitchens is lowered into the container. The "Mix Master" stirrer is the product of and obtainable from the Chicago Flexible Shaft Co., 1124 South Central Avenue, Chicago, Illinois. The stirring elements are similar in construction and action to the familiar household egg beater, consisting of two shafts oppositely rotated by a motor, and two elliptical loops attached to each shaft, one loop being at right angles to the other and the two loops having a common long axis. The dimensions and form of the vessel and stirring elements will be better understood, and can be duplicated by, reference to Figs. 2 and 3.

Fig. 2 shows, partly in cross section and partly in front elevation, the container and the stirring elements, while Fig. 3 shows in front elevation a detailed view of one-half of one loop of one stirring element.

Referring to Fig. 2, the apparatus comprises a cylindrical flat bottomed container I and two stirring elements II constructed exactly alike. The internal dimensions of the container, as shown, are a diameter of 6" and a height of 5". The stirring elements consist each of an upper shaft A geared at the top to a motor (not shown) and rigidly secured at the bottom to a lower shaft B and to two elliptical loops C and D which are disposed at right angles to each other and have each the shaft B as their long axis and as a supporting member. Shaft B is rigidly secured to the tops and bottoms of loops C and D. In the preferred construction, as shown, shaft A is sturdier than shaft B, but this is not necessary; for example, a single shaft of uniform diameter may take the place of shafts A and B, passing through the tops of loops C and D and being secured thereto at the top and bottom of the loops. The stirring elements II are so placed in vessel I that shafts A are parallel and 1 1/8" apart (center to center) and they are placed in vessel I so that a line drawn half way between and in the plane of the shafts coincides with the axis of vessel I, and the distance from the bottom of loops C to the bottom of vessel I is 1/4 inch. The shafts A are so geared to the motor that they rotate at equal speeds in opposite directions.

Referring to Fig. 3, shafts A and B and one-half of loop C are shown. The other half of loop C, and both halves of loop D are identically constructed.

Shaft B is cylindrical and has a diameter of  $\frac{1}{4}$ " and a length of  $3\frac{3}{8}$ ". Loop C consists of a flat strip of metal or equivalent material  $\frac{1}{2}$ " thick and  $\frac{1}{4}$ " wide. It is bent approximately in the shape of an ellipse with a short radius of  $1\frac{1}{4}$ ". It has flat sides  $1\frac{3}{4}$ " long, and the portions between the flat sides and shaft B have approximately the curvature of a circle.

Small variations of the structure of the loop and of the diameter of shaft B may be made without altering substantially the results obtained.

In operation, the oil in container I is maintained at 275° F. and stirring elements A are rotated in opposite directions each at the rate of 1100 revolutions per minute. The volume increase due to foaming is determined by measuring the height of the oil before foam formation and after foam formation.

We claim:

1. A foam inhibited mineral oil, comprising a major quantity of an excessively foaming mineral oil of lubricating viscosity, and a minor quantity, sufficient to inhibit foaming, of a compound which contains not less than about 15 per cent by weight of oxygen, has a molecular weight not higher than about 270, and is represented by the formula  $A(X)_a(OR)_b$  wherein A is an aromatic nucleus, X is an oxygen-containing substituent, R is a member of the class consisting of hydrogen, alkyl, cycloalkyl, aryl and aralkyl radicals, and a and b are integers.

2. A foam inhibited mineral oil, comprising a major quantity of an excessively foaming mineral oil of lubricating viscosity, and a minor quantity, sufficient to inhibit foaming, of a compound which contains not less than about 15 per cent by weight of oxygen, has a molecular weight not higher than about 270, and is represented by the formula  $A(X)_a(OR)_b$  where A is a benzene nucleus, X is a carbon- and oxygen-containing substituent, R is a member of the class consisting of hydrogen, alkyl, cycloalkyl, aryl and aralkyl radicals, and a and b are integers.

3. A foam inhibited mineral oil, comprising a major quantity of an excessively foaming mineral oil of lubricating viscosity, and a minor quantity, sufficient to inhibit foaming, of a compound which contains not less than about 15 per cent by weight of oxygen, has a molecular weight not higher than about 270, and is represented by the formula

$A(X)_a(OR)_b$

wherein A is a benzene nucleus, X is a substituent containing carbonyl oxygen, R is a member of the class consisting of hydrogen, alkyl, cycloalkyl, aryl, and aralkyl, and a and b are integers.

4. A foam inhibited mineral oil, comprising a major quantity of an excessively foaming mineral oil of lubricating viscosity and a minor quantity, sufficient to inhibit foaming, of a compound which contains not less than about 15 per cent by weight of oxygen, has a molecular weight not higher than about 270, and is represented by the formula

$A(X)_a(OR)_b$

wherein A is a benzene nucleus, X is a carboxy ester substituent, R is a member of the class consisting of hydrogen, alkyl, cycloalkyl, aryl, and aralkyl, and a and b are integers.

5. In the lubrication of machinery at oil temperatures above about 150° F. with compounded mineral oil lubricants which tend to foam exces-

sively, and under conditions of oil agitation and intermixture with gas which tend to cause excessive foaming, the method of inhibiting foaming of the lubricating oil, which comprises maintaining therein a small amount, sufficient to inhibit foaming, of a substituted aromatic compound containing not less than about 15 per cent by weight of oxygen, containing at least two oxygen atoms and having a molecular weight not higher than about 270.

6. A foam inhibited lubricating oil, comprising an excessively foaming hydrocarbon lubricating oil and a small amount, sufficient to inhibit foaming of the oil, of an aromatic compound of molecular weight not greater than about 270, containing at least two oxygen atoms and containing not less than about 15% by weight of oxygen.

7. A foam inhibited lubricating oil, comprising an excessively foaming hydrocarbon lubricating oil and a small amount, sufficient to inhibit foaming of the oil, of an aromatic compound of molecular weight not greater than about 270, containing at least two oxygen atoms, containing not less than about 15% by weight of oxygen and consisting of nonmetallic elements.

8. The oil of claim 7, wherein said aromatic compound is present in the oil in the amount of about 0.001 to 0.1 per cent by weight based on finished oil.

9. A foam inhibited lubricating oil, comprising an excessively foaming petroleum lubricating oil and a small amount, sufficient to inhibit foaming of the oil, of a compound, selected from the group consisting of derivatives of benzene and derivatives of naphthalene, said compound having a molecular weight not greater than about 270, containing at least two oxygen atoms, containing not less than about 15% by weight of oxygen and consisting of carbon, hydrogen and oxygen.

10. The oil of claim 9, wherein said compound is present in the oil in the amount of about 0.001 to 0.1 per cent by weight based on finished oil.

11. The oil of claim 9, wherein said compound is saligenin.

12. The oil of claim 9, wherein said compound is methyl salicylate.

13. The oil of claim 9, wherein said compound is benzoyl acetone.

14. A compounded lubricating oil comprising a hydrocarbon base oil, at least one salt selected from the group consisting of oil-soluble metal salts of organic acids and oil-soluble metal salts of organo-substituted inorganic acids, and a small amount, sufficient to inhibit foaming of the oil, of an aromatic compound of molecular weight not greater than about 270, containing at least two oxygen atoms and containing not less than about 15% by weight of oxygen.

15. A compounded lubricating oil comprising a hydrocarbon base oil, at least one salt selected from the group consisting of oil-soluble metal salts of organic acids and oil-soluble metal salts of organo-substituted inorganic acids, and a small amount, sufficient to inhibit foaming of the oil, of an aromatic compound of molecular weight not greater than about 270, containing at least two oxygen atoms, containing not less than about 15% by weight of oxygen and consisting of nonmetallic elements.

16. A compounded lubricating oil comprising a petroleum lubricating oil, a foam-promoting amount of at least one salt selected from the group consisting of oil-soluble polyvalent metal salts of organic acids and oil-soluble polyvalent metal salts of organo-substituted inorganic acids,

said oil-soluble polyvalent metal salts being salts which promote foaming of the oil when the oil is subjected to violent intermixture with air, and a small amount, sufficient to inhibit foaming of the oil, of a compound selected from the group consisting of derivatives of benzene and derivatives of naphthalene, said compound having a molecular weight not greater than about 270, containing at least two oxygen atoms and consisting of carbon, hydrogen and oxygen.

17. A compounded lubricating oil comprising a petroleum lubricating oil, an oil-soluble polyvalent metal phenate and a small amount, sufficient to inhibit foaming of the oil, of an aromatic compound having a molecular weight not greater than about 270, containing at least two oxygen atoms, containing not less than about 15% by weight of oxygen and consisting of non-metallic elements.

18. A compounded lubricating oil comprising a petroleum lubricating oil, an oil-soluble polyvalent metal organo phosphate and a small amount, sufficient to inhibit foaming of the oil, of an aromatic compound having a molecular weight not greater than about 270, containing at least two oxygen atoms, containing not less than about 15% by weight of oxygen and consisting of non-metallic elements.

19. A compounded lubricating oil comprising a petroleum lubricating oil, a small amount each, sufficient to stabilize the oil and to inhibit piston discoloration and piston ring sticking in an internal combustion engine, of an oil-soluble polyvalent metal phenate and an oil-soluble polyvalent metal organo phosphate, and a small amount, sufficient to inhibit foaming of the oil, of an aromatic compound having a molecular weight not greater than about 270, containing at least two oxygen atoms, containing not less than about 15% by weight of oxygen and consisting of non-metallic elements.

20. A compounded liquid lubricant comprising a major proportion of a petroleum lubricating oil containing an oil-soluble foam-promoting metal salt in an amount sufficient substantially to increase the tendency of the lubricating oil to foam excessively at temperatures above about 150° F. and under conditions of severe oil agitation and intermixture with gas, and a minor amount, sufficient substantially to inhibit the said excessive foaming, of a compound which contains not less than about 15 per cent by weight of oxygen, has a molecular weight not higher than about 270, and is represented by the formula  $A(X)_a(OR)_b$  wherein A is an aromatic nucleus, X is an oxygen-containing substituent, R is a member of the class consisting of hydrogen, alkyl, cycloalkyl, aryl and aralkyl radicals, and  $a$  and  $b$  are integers.

VICTOR N. BORSOFF.  
JAMES O. CLAYTON.

#### REFERENCES CITED

The following references are of record in the  
25 file of this patent:

#### UNITED STATES PATENTS

| Number     | Name      | Date           |
|------------|-----------|----------------|
| 2,261,047  | Aneff     | Oct. 28, 1941  |
| 2,031,986  | Stratford | Feb. 25, 1936  |
| Re. 22,189 | Prutton   | Sept. 29, 1942 |
| 2,298,465  | Clapsadle | Oct. 13, 1942  |
| 1,826,897  | Rice      | Oct. 13, 1931  |
| 1,981,506  | Hansen    | Nov. 20, 1934  |
| 2,045,551  | Iddings   | June 23, 1936  |
| 2,134,554  | Grobel    | Oct. 25, 1938  |
| 2,215,590  | Maverick  | Sept. 24, 1940 |
| 2,320,263  | Carlson   | May 25, 1943   |
| 2,134,736  | Reuter    | Nov. 1, 1938   |
| 2,145,971  | Cantrell  | Feb. 7, 1939   |
| 2,216,711  | Musher    | Oct. 1, 1940   |

#### Certificate of Correction

Patent No. 2,430,857.

November 18, 1947.

VICTOR N. BORSOFF ET AL.

It is hereby certified that error appears in the printed specification of the above numbered patent requiring correction as follows: Column 3, in the fourth formula, for



read



and that the said Letters Patent should be read with this correction therein that the same may conform to the record of the case in the Patent Office.

Signed and sealed this 27th day of January, A. D. 1948.

[SEAL]

THOMAS F. MURPHY,  
Assistant Commissioner of Patents.